

## UNITED STATES PATENT OFFICE.

EDDIE LAMBERT AND WALTER E. MATHEWS, OF BALTIC, CONNECTICUT.

## PROCESS OF PRODUCING PAPER PULP.

No Drawing.

Application filed August 26, 1922. Serial No. 584,571.

*To all whom it may concern:*

Be it known that we, EDDIE LAMBERT and WALTER E. MATHEWS, citizens of the United States, residing at Baltic, in the county 5 of New London and State of Connecticut, have invented certain new and useful Improvements in Processes of Producing Paper Pulp, of which the following is a specification.

10 This invention relates to a process of treating wood pulp for employment in the manufacture of paper. Heretofore it has been found practical to employ only certain kinds of wood such, for example, as spruce, 15 hemlock, and poplar, it being customary, furthermore, to carefully select the stock. As this necessity for selection of certain kinds and grades of wood is the chief item 20 of expense in the manufacture of paper, the present invention has as its object to evolve a process of treatment of any and all kinds of wood for the preparation of pulp which may be successfully employed 25 in the manufacture of a reasonably good quality of paper.

In carrying out the invention stock of any kind of wood in a more or less divided state as, for example, in the form of chips or sawdust is comminuted in a grinding 30 machine of any approved type. The ground fibrous mass is then boiled in a solution of an alkali such as caustic potash for a period of about one hour, it being preferable to

employ about one pound of the alkali with sufficient water to cover approximately one 35 hundred pounds of the fibrous material. In this step the fibers are softened and separated, and all resinous matters are removed.

The pulpy mass produced in accordance with the foregoing step is then washed with 40 water to remove all dirt and foreign matter, and is next ground again, and if desired finally bleached by any suitable agent such, for example, as chloride of lime. The 45 pulp is then ready for use in the manufacture of paper.

It has been found that by carrying out this process it is possible to make use of practically any kind of wood, and the product is a highly desirable one.

Having thus described the invention, what is claimed as new is:

The process of treating wood stock for the preparation of paper pulp which comprises comminuting the stock, boiling the 55 same for a period of approximately one hour in a solution of one pound of caustic potash in sufficient water to cover approximately one hundred pounds of the stock, washing the stock to remove the dirt, and re-grinding the cleansed stock.

In testimony whereof we affix our signatures.

EDDIE LAMBERT. [L. S.]  
WALTER E. MATHEWS. [L. S.]